

Patented Oct. 2, 1928.

1,686,149

# UNITED STATES PATENT OFFICE.

GEORGE HOLLAND ELLIS, OF SPONDON, NEAR DERBY, ENGLAND, ASSIGNOR TO CELANESE CORPORATION OF AMERICA, A CORPORATION OF DELAWARE.

## TREATMENT OF FABRICS.

No Drawing. Application filed December 3, 1926, Serial No. 152,515, and in Great Britain July 27, 1926.

This invention relates to the treatment of woven, knitted or other fabrics and especially fabrics made with or containing threads or yarns composed of or comprising 5 filaments or fibres of cellulose acetate or other cellulose esters or cellulose ethers,—for the purpose of rendering them less liable to or immune from development of faults caused through lack of cohesion or low coefficient of friction existing between the 10 threads or yarns of the fabrics at their points of crossing or interlooping.

In the case of woven fabrics these faults are commonly referred to as "slipping", the 15 term indicating that stresses in usage or in processes subsequent to weaving cause the threads of one component (i. e. the warp or weft) to slip over those of the other and produce, at the point of slipping, uneven 20 distribution of the warp threads or weft threads. The fault is least observable in closely woven fabrics having a high number of reed and pick, and is most likely to occur in fabrics with a small number of crossings 25 (i. e. points of contact of warp and weft) per unit area.

In the case of circular knitted fabrics or other weft-knitted fabrics the fault is commonly known as "laddering" and is caused 30 by a line or series of loops in the fabrics (on breakage of a loop or thread) becoming drawn out of or slipping out of the adjacent loops through which they are threaded in the structure of the fabric, owing to lack 35 of cohesion or low coefficient of friction at the points of contact of the loops, so that a ladder-like defect results; while in the case of warp-knitted fabrics the fault is commonly known as "splitting" and is produced by 40 the fabric splitting continuously along a wale of the fabric without tearing if a cut happens to be made lengthwise in the middle of the wale in a direction towards the beginning of the fabric, such splitting being 45 likewise due to lack of cohesion or low coefficient of friction existing between the threads of the fabric.

It has now been found that by subjecting woven, knitted or other fabrics,—and especially fabrics made with or containing threads or yarns composed of or comprising filaments or fibres of cellulose acetate or other cellulose esters or cellulose ethers,—to the process of the present invention, their tendency to develop the faults of the character

referred to is greatly minimized or even eliminated.

The precise reason for the efficacy of the process of the present invention is not entirely clear, but it may possibly be due to the penetrative or "wetting out" properties of the substances applied as hereinafter described, whereby the filament or fibre units of the yarns (by this penetration of the interstices as well as of their own substances) 60 are possibly opened out and swollen in a manner which increases the binding power of the threads or yarns to produce a more 65 resistant fabric.

According to the present invention, for 70 the purpose referred to, woven, knitted or other fabrics,—and especially fabrics made with or containing yarns or threads composed of or comprising filaments or fibres of cellulose acetate or other cellulose esters or 75 cellulose ethers,—are subjected to simple or repeated application, by impregnation with strong aqueous solutions or dispersions of one or more bodies known to have a solubilizing or dispersing power for water-insoluble or relatively water-insoluble dyestuffs, that is to say a power of rendering water-insoluble or relatively water-insoluble dyestuffs soluble or capable of high dispersion 80 in water. In the subsequent description and 85 claims such bodies are referred to as dispersing agents and their aqueous solutions and dispersions are referred to collectively as aqueous solutions.

The following are examples of such dispersing agents:—sulphorcinoleic acid or other sulphated fatty acids or other bodies having oily or fatty characteristics, namely oleic, stearic, palmitic, and the other higher fatty acids and sulphonated or other derivatives thereof containing salt-forming groups (e. g. the sulpho group or the carboxyl group or both sulpho and carboxyl groups) and soluble salts of such acids or derivatives, for instance their alkali or ammonium salts or mixtures of two or more of such acids and/or derivatives and/or salts; for the sake of brevity all such acids, derivatives and salts and mixtures are herein included in the term body of oily or fatty 95 characteristics.

Carbocyclic compounds containing in their structure one or more salt-forming groups (such as sulphonate, carboxyl or hydroxyl groups), whether the compound contains 100 110

only one kind of these groups or different kinds of these groups at the same time—and sodium or other soluble salts of said compounds; or mixtures of any of such carbocyclic compounds and/or salts, or mixtures of one or more thereof with one or more of the aforesaid bodies of oily or fatty characteristics. As instances of said carbocyclic compounds and salts may be mentioned 5 naphthenic acids, naphthene sulphonic acids, or other carboxylic or sulphonic acids of the cycloparaffins; phenols, sulphonic acids, carboxylic acids, phenolsulphonic acids or other derivatives of the benzene, naphthalene or 10 anthracene series containing one or more salt forming groups, or other derivatives of saturated or non-saturated cyclic hydrocarbons containing one or more salt-forming groups, and sodium or other soluble salts of 15 any of these compounds.

20 Sulpho aromatic fatty acids, such for instance as sulpho-benzene stearic acid, (Twitchell reagent), or derivatives thereof such as sulphophenol stearic acid, sulpho- 25 napthalene stearic acid, sulphobenzeno-ericinoleic acid, sulphophenolricinoleic acid, sulphonaphthalene ricinoleic acid, or sodium or other soluble salts of such acids or derivatives, or mixtures of any of such and/or 30 derivatives and/or salts.

Soluble resin soaps, or sodium or other soluble salts or soaps of resin acids.

35 For the purpose of the present invention it has been found that, of the dispersing agents hereinbefore referred to, the salts and the mixtures of the free acids or salt-forming compounds with the salts whether of the same or of different acids or salt forming compounds are especially useful.

40 In carrying out the process of the present invention the goods may be subjected to the impregnation by any suitable means, but I have found the machine known as the padding mangle to be particularly suitable. This apparatus provides for the passage of 45 the fabric through the strong aqueous solution of one or more dispersing agents, followed by a squeeze between rollers, so that excess of liquor is expressed, rendering subsequent rolling up or other manipulation more easy. The aqueous solutions may be 50 applied at any suitable temperatures and concentrations, but I have found the best results to be achieved with hot liquors at 55 about 80° C., or, where the fabric will withstand them—boiling temperatures. Further, I have found that the most favorable results are obtained when employing the dispersing agents in concentrations of over 60 about 10%; and that especially favorable results are obtained when employing, for the purpose of the present invention, aqueous solutions or dispersions of sodium or potassium salts of oleic, palmitic, stearic, ricinoleic or like fatty acids, or of the sulphated

fatty acids such as the well known Turkey red oil of commerce, the last named being very effective.

70 After the impregnation and squeeze, the goods are preferably piled or rolled up to avoid evaporation and cooling and left for a number of hours, conveniently overnight in commercial working, then after this "maturing" period, scoured as desired, and dried, or passed direct to any such subsequent processing as dyeing or printing. The impregnation process may be repeated in which case after scouring off the first time, the fabric is preferably dried in open width, as 75 for instance on the well known continuous tentering machine, before the second impregnation.

80 The following example of one practical form of execution will serve to illustrate how the invention may be carried out, it being understood that this is given by way of illustration only and is in no way limitative.

*Example.*

85 40 kgr. of a fabric woven of artificial silk 90 warp and weft (for instance cellulose acetate artificial silk) are impregnated in a padding mangle with a Turkey red oil solution of 45% fatty acid content. The squeeze rollers are applied so as to leave in the fabric about 20 kgr. of the solution which shows a temperature of 80° C. during the application. The fabric is batched or rolled up on a suitable roller and left overnight. The next day the fabric is scoured in open width in a solution of sodium oleate of 5 grams per litre strength at 75° C. for one hour, for example on the "jigger" machine familiar in the dyeing arts. It is afterwards well rinsed, hydro-extracted and dried on the continuous 100 clip tenter. The impregnation process is repeated exactly, followed by the "maturing" 105 period and scour; the goods are then passed to dyeing and printing or other process, or are immediately "finished" as desired. The 110 tendency to slip will be found to have been eliminated or much minimized.

115 It is to be understood that fabrics which have been found to show liability to the "slipping," "laddering" or "splitting" defects after processing such as dyeing, may be subjected to the above described processes for preventive or ameliorative treatment in respect of this liability.

120 While the process of the present invention is of especial value for treating fabrics made with or containing yarns or threads composed of or comprising filaments or fibres of cellulose all of which are hereinafter in the claims referred to as fabrics comprising organic substitution derivatives of cellulose acetate or other esters or ethers of cellulose, it may with advantage be applied to fabrics made with or containing yarns or threads composed of or comprising other filaments 125

- or fibres, for instance natural silk, artificial silks of the cellulosic type, (e. g. cuprammonium silk, viscose silk, "nitrocellulose" silk and the like), cotton, wool and so forth.
5. What I claim and desire to secure by Letters Patent is:—
1. Process for the treatment of fabrics to render them less liable to develop faults, comprising impregnating the fabrics with strong aqueous solutions of dispersing agents.
  2. Process for the treatment of fabrics to render them less liable to develop faults, comprising impregnating the fabrics with aqueous solutions of dispersing agents of at least 10% strength.
  3. Process for the treatment of fabrics comprising organic substitution derivatives of cellulose to render them less liable to develop faults, comprising impregnating the fabrics with strong aqueous solutions of dispersing agents.
  4. Process for the treatment of fabrics comprising organic substitution derivatives of cellulose to render them less liable to develop faults, comprising impregnating the fabrics with aqueous solutions of dispersing agents of at least 10% strength.
  5. Process for the treatment of fabrics comprising organic substitution derivatives of cellulose to render them less liable to develop faults, comprising impregnating the fabrics with strong aqueous solutions of dispersing agents and batching them for a predetermined time.
  6. Process for the treatment of fabrics comprising organic substitution derivatives of cellulose to render them less liable to develop faults, comprising impregnating the fabrics with strong aqueous solutions of bodies of oily or fatty characteristics.
  7. Process for the treatment of fabrics comprising organic substitution derivatives of cellulose to render them less liable to develop faults, comprising impregnating the fabrics with aqueous solutions of at least 10% strength of bodies of oily or fatty characteristics and batching them for a predetermined time.
  8. Process for the treatment of fabrics comprising organic substitution derivatives of cellulose to render them less liable to develop faults, comprising impregnating the fabrics with an aqueous solution of at least 10% strength of a sulphonated fatty acid compound and batching them for a predetermined time.
  9. Process for the treatment of fabrics comprising cellulose acetate to render them less liable to develop faults, comprising impregnating the fabrics with strong aqueous solutions of dispersing agents.
  10. Process for the treatment of fabrics comprising cellulose acetate to render them less liable to develop faults, comprising impregnating the fabrics with aqueous solutions of dispersing agents of at least 10% strength.
  11. Process for the treatment of fabrics comprising cellulose acetate to render them less liable to develop faults, comprising impregnating the fabrics with strong aqueous solutions of dispersing agents and batching them for a predetermined time.
  12. Process for the treatment of fabrics comprising cellulose acetate to render them less liable to develop faults, comprising impregnating the fabrics with strong aqueous solutions of bodies of oily or fatty characteristics.
  13. Process for the treatment of fabrics comprising cellulose acetate to render them less liable to develop faults, comprising impregnating the fabrics with aqueous solutions of at least 10% strength of bodies of oily or fatty characteristics and batching them for a predetermined time.
  14. Process for the treatment of fabrics comprising cellulose acetate to render them less liable to develop faults, comprising impregnating the fabrics with an aqueous solution of at least 10% strength of a sulphonated fatty acid compound and batching them for a predetermined time.
  15. Process for the treatment of fabrics comprising cellulose acetate to render them less liable to develop faults, comprising impregnating the fabrics with strong aqueous solutions of Turkey red oil.
  16. Process for the treatment of fabrics comprising cellulose acetate to render them less liable to develop faults, comprising impregnating the fabrics with aqueous solutions of Turkey red oil of at least 10% strength and batching them for a predetermined time.
  17. Process for the treatment of fabrics comprising cellulose acetate to render them less liable to develop faults, comprising impregnating the fabrics with a Turkey red oil solution of 45% fatty acid content, batching for a predetermined time and then scouring.
- In testimony whereof I have hereunto subscribed my name, this 12th day of November, 1926.

GEORGE HOLLAND ELLIS.